

## UNITED STATES PATENT OFFICE

2,423,314

AGGLOMERATION BY SULFONATED RE-  
AGENTS IN MAGNETIC RECOVERY OF  
IRON ORESEarl Conrad Herkenhoff, Stamford, Conn., as-  
signor to American Cyanamid Company, New  
York, N. Y., a corporation of MaineNo Drawing. Application June 1, 1945,  
Serial No. 597,146

7 Claims. (Cl. 209—8)

1

This invention relates to the beneficiation of mineral values of low grade iron ores by a novel combination of chemical pretreatment and magnetic separation. Broadly, the process is applicable to the beneficiation of oxide minerals from iron ores containing an excess of acidic or silicious gangue. More particularly, the invention is especially well adapted to the treatment of ores in which a non-magnetic oxide constituent occurs with a magnetic or a magnetizable oxide constituent.

Increasing amounts of various lower grade ores are becoming industrially important because of the decreasing supply of high grade ores. Typical illustrations are found in iron ores. Many deposits comprise ores which are too low in iron and too high in silico-bearing gangue to be suitable for use as blast furnace feed. To be useful they must be beneficiated in some manner. Calcium carbonate and other alkaline earth oxide and carbonate minerals also frequently occur in other iron ores. These may be even to a certain extent desirable, but if the iron content is too low, it must be raised by removing a portion of these minerals. The problem, then, is one reducing impurities and raising the mineral value content to as high a degree as practicable.

Beneficiation has been attempted by many different procedures, depending upon the ore. In some cases the necessary increases in grade may be made simply by crushing and washing the ore. Where the mineral values and the gangue are associated in such manner that this cannot be done, the mineral values must be released by crushing or grinding. Heavy-media separation has proved particularly useful in the treatment of particle sizes down to about  $\frac{1}{16}$  inch. Other naturally occurring ores require reduction to smaller sizes, as low as 35-48 mesh down to fines, to unlock the objectionable gangue, and various froth flotation procedures have been developed for use in beneficiating these finely ground ores. It is with those ores which must be reduced to 8-12 mesh or smaller that the present invention is particularly concerned.

In the past it has been proposed to beneficiate finely ground, low-grade, non-magnetic ores by magnetic treatment rather than by froth flotation. Perhaps the best of such processes consists in mixing magnetically-susceptible particles

2

with a ground ore of non-magnetic minerals and treating an aqueous pulp of these mixtures with a fatty acid, such as oleic acid, apparently to distribute a film of finely divided magnetic particles over the surface of the non-magnetic particles. The treated pulp is then usually deslimed, at least the sands are dried and the dried material subjected to magnetic separation, the magnetically susceptible portion being thereby withdrawn and carrying with it the non-magnetically susceptible material associated therewith. This procedure is of little use except in conjunction with flotation or some similarly more effective operation. When used alone it does not give either a particularly good recovery or a particularly good degree of concentration. It is also subject to several other objections in that it involves separation of sands and slimes and that it requires a drying operation before treating by dry magnetic separation.

Nevertheless, a practicable magnetic separation is commercially very desirable. For treating many ores, it would possess definite advantages over froth flotation, both technically and economically. It is, therefore, the principal object of the present invention to develop a magnetic beneficiating process which is not subject to the objectionable features noted above.

Because many iron ores naturally occur as admixtures of non-magnetic iron oxides, such as hematite, magnetite and the like, with such magnetic oxides as magnetite, the process will be discussed in connection therewith. In general, the desired object is obtained by treating an aqueous pulp of the ore with a suitable sulfonated agglomerating agent and then subjecting the conditioned pulp directly to magnetic separation. This eliminates much of the subsequent desliming problem and the necessity for drying as is taught in the prior art. Equally important, if not more so, the process when used alone yields products which are satisfactory in both grade and recovery.

According to the present invention the sulfonated agglomerating agents which may be used in accordance therewith may be quite widely varied. Among the various reagents suitable for the purpose are such materials as the sulfonated petroleum hydrocarbons, both the so-called water-soluble "green" acid and oil-soluble "mahogany" acid types obtained in the refining of petroleum

lubricating oils; sulfonated fatty acids, such as lauric, oleic, linoleic, cocoanut fatty acids, soya-fatty acids and the like; sulfonated abietic acids; sulfonated naphthenic acids; such sulfonated, saponifiable oils, i. e., esters of polyhydric alcohols and long chain aliphatic acids of animal and vegetable origin, as corn oil, fish oil, cottonseed oil, palm oil, and the like; sulfonated crude and refined talloel and mixtures thereof, also sulfonated, organic residues as still bottoms, pitches, distillation by-products, oils recovered from various processes and the like.

Throughout this case in referring to "petroleum sulfonates," the terms "sulfonate" and "sulfonated" are used very loosely. Many of these products are mixtures of indeterminate chemical constitution and often a large portion of the combined acid groups are actually sulfate groups rather than sulfonic acid groups. This is largely due to their original which, as noted above, is in the refining of petroleum lubricating oil stocks. As shown for example in U. S. Patent 2,331,049, their principal source is as by-products from the refining of petroleum lubricating oil fractions in the course of treatment with fuming sulfuric acids or sulfuric acids. Hence, the terms will be used not in their strict chemical sense but in the general sense in which they are employed in the art.

These sulfonated reagents may be used in neutral or alkaline circuit if so desired, in which case suitable alkaline conditioning or modifying agents, such as soda ash, caustic soda, sodium silicate, and the like, may be added. However, most of the problems which the present invention was designed to overcome are present in the beneficiation of many iron ores, and the best results with such ores appear to be obtained in acidic circuit. That consideration must also be applied. Almost any acidic agent, which is itself or yields a product which is an acid having a fairly high dissociation constant, preferably greater than about  $10^{-7}$ , may be used. For practical purposes, sulfuric acid, because of its low cost and availability, is an acidic material which is attractive from a commercial point of view. Ordinarily, a sufficient amount should be used so that a pH of between about 5.5 and 1.5 is produced.

Conditioning with the reagents, which is an important feature of the present invention, often presents a problem of physical distribution. This is particularly acute both where the reagent is not readily dispersible in water and where the collector is very soluble. In such cases an oiling agent may profitably be used as an adjunct. Unsaponifiable hydrocarbon oils such as fuel oil give excellent results and their low price makes them very attractive in most locations. In practice they are to be preferred. However, other oils such as glyceride oils, for example, cocoanut oil, linseed or cottonseed oils, can be made to work satisfactorily. Certain fatty acids of oily nature if necessary also may be used in acid circuit. The amount of oiling, however, depends very largely on the particular reagents used and may vary from a small amount up to several pounds per ton. With every reagent combination there is an optimum range of oiling agent. This range is not critical and is not the same in every case. The optimum proportions should be determined in each case, but once determined, no operating difficulties result since the range is broad enough to take care of ordinary fluctuations in operation.

In general, the principal process steps of the

present invention are exceedingly simple. While the overall procedure may be varied, several steps are characteristic. First, if the ore contains no magnetically susceptible material, the latter must be provided. Second, an aqueous pulp of the ore, previously reduced to a sufficient fineness to liberate essentially the mineral values, is conditioned to cause agglomeration of the magnetically susceptible and the desired non-magnetically susceptible material. Third, the conditioned pulp is, without other treatment, subjected to a strong magnetic influence whereby the agglomerated or flocculated material is drawn therefrom.

The second and third steps are always present whether the ore is one which naturally contains material of high coercive force and remanence or whether such material is artificially incorporated therein. They constitute common features between such processes and those in which the magnetic and non-magnetic mixture constitutes the desired concentrate, in which the magnetic material is subsequently separated from the non-magnetic portion, which itself is the desired concentrate, and those in which the magnetic material is separated and reused. The process may be applied not only to naturally-occurring ores but also to products from previous beneficiation such as tabling, flotation and the like.

As has been noted, the process requires chemical treatment of the ore in an aqueous pulp. The extent to which the ore is reduced in size before pulping is determined largely by the degree of crushing or grinding required to free the mineral values. The process is not limited to the relatively fine grinding normally required for froth flotation. It can be applied to particle sizes which are too small for efficient beneficiation by heavy-media separation but too large for froth flotation: i. e., minus 8 plus 35 mesh. It can also be used in the size range usually handled in froth flotation processes, i. e., minus 35-48 mesh to fines. Thus the present process is applicable to a wider range of particle sizes than is a conventional process of froth flotation. In addition, it is simply and readily operated, normally requires less apparatus and is more economical in operation.

The problem of slime is not greatly different than in froth flotation processes. In the case of the present invention, as elsewhere, slime is never desirable. However, it is an advantage that the agglomerating agents may be chosen from a wide variety, some of which are less affected by slimes than others. Thus it is possible to treat undeslimed ores, partially deslimed and thoroughly deslimed ores, the choice depending upon various factors. The effect of slimes is noticeable primarily in added consumption of the agglomerating agent. As the preferable agents of this invention are not expensive, it may be advantageous to not deslime or to remove only the colloidal fractions and use more reagents. The extent of desliming is therefore one of economic compromise and must be determined in the case of each ore.

So far as the efficiency of the chemical pre-treatment is concerned, it may be carried out in pulps of either low or high density. The choice may vary somewhat with the chemical agents used but actually depends principally on the apparatus used. Conditioning may be carried out in a type of rolling drum, or an open tank having a mechanical impeller therein, or any other apparatus capable of efficient mechanical agitation and mixing. The use of a tank and impeller, for

example, permits treating pulps of high solids content, i. e., 50-70%, or more solids. With many reagents, this practice may give a better dispersion of the reagents over the solids in the pulp. It also requires less equipment since the volumes to be handled are smaller.

On the other hand, it may be desirable to condition the pulp in an agitator similar in construction to the conventional, mechanical type flotation machine such as the well-known Fagergren or Denver cells. This ordinarily requires pulps of low density, usually 25% or less solids. This, except for the necessity of handling larger pulp volumes, is not particularly disadvantageous since most of the preferred reagents are about equally effective when conditioned at either high or low solids.

On the other hand, the disadvantage in handling larger pulp volumes may be often far more than offset by the advantage of being able to introduce small amounts of fine air bubbles into the pulp during agitation. Presumably each small discrete air bubble becomes surrounded with treated particles, thus assisting in agglomeration of the magnetic and non-magnetic material. This should not be confused with the frothing produced by purposely introducing large volumes of air during froth flotation operations. The amount of air introduced according to the present process is only a fraction of that used in ordinary practice of froth flotation. Because of the extremely minute air bubbles which it is capable of introducing, a conditioner employing the Fagergren type rotor and stator is preferable for this purpose.

After being conditioned with the agglomerating agent, the conditioned pulp is then subjected to magnetic separation. This can be carried out in any of a number of conventional machines which are commercially available for the purpose; for example, the well known Steffensen and Crockett separators. No particular precautions are ordinarily necessary except that in those cases where the conditioning step is carried out at very high solids, it is usually desirable to dilute

25

30

35

40

45

was made directly into an aqueous pulp of about 25% solids and subjected directly to magnetic separation. Further, in order to show the ineffectiveness of carrying out a conditioning step with a fatty acid as taught by the prior art, the second sample was treated in the same way except that before the magnetic treatment the pulp was conditioned for two minutes with 2 lbs./ton of oleic acid. From the results shown in the following Table I, it will be noted that this procedure gives a slightly poorer grade and very little better recovery than when the step was omitted entirely.

Table I

| Test No. | Product     | Per cent Weight | Assay, per cent |        | Per cent Distrib. of Fe |
|----------|-------------|-----------------|-----------------|--------|-------------------------|
|          |             |                 | Fe              | Insol. |                         |
| 1.       | Head        | 100.00          | 55.00           | 19.36  | 100.00                  |
|          | Concentrate | 41.99           | 67.30           | 3.56   | 51.38                   |
|          | Tailing     | 38.01           | 46.10           | 30.80  | 48.62                   |
| 2.       | Head        | 100.00          | 54.67           | -----  | 100.00                  |
|          | Concentrate | 48.84           | 65.82           | 3.72   | 58.79                   |
|          | Tailing     | 51.16           | 44.03           | -----  | 41.21                   |

## EXAMPLE 2

In order to show the comparative effectiveness of conditioning with the reagents of the present invention rather than the fatty acid of the prior art, a number of additional samples of the same ore used in Example 1 were treated according to the process of the present invention by conditioning an aqueous pulp of the ore containing about 70% solids for 2 minutes with the reagents, diluting the pulp to about 25% solids, and then subjecting the pulp to magnetic separation. The reagents used and the metallurgical results obtained are shown in Table II. It will be seen that whereas the grade is substantially that obtained when no conditioning step is used, as in the case of Test 1 of Example 1, the recovery was increased as much as 50 to 65%. This increase in recovery is very important since the improvement represents entirely an increase in ordinarily non-magnetically susceptible iron minerals.

Table II

| Test No. | Product     | Per Cent Wt. | Assay, Per Cent |        | Distrib. Per Cent Fe | Reagents |                                    |
|----------|-------------|--------------|-----------------|--------|----------------------|----------|------------------------------------|
|          |             |              | Fe              | Insol. |                      | Lbs./ton | Type                               |
| 1.       | Head        | 100.00       | 54.95           | -----  | 100.00               | 2.0      | Sulfuric acid.                     |
|          | Concentrate | 74.24        | 65.74           | 3.62   | 88.82                | 2.8      | Oil-soluble petroleum sulfonate.   |
|          | Tailing     | 25.76        | 23.86           | -----  | 11.18                | 3.9      | Fuel oil, 22° Bé.                  |
| 2.       | Head        | 100.00       | 54.84           | -----  | 100.00               | 1.5      | Sulfuric acid.                     |
|          | Concentrate | 59.13        | 65.36           | 4.14   | 70.48                | 2.8      | Water-soluble petroleum sulfonate. |
|          | Tailing     | 40.87        | 39.60           | -----  | 29.52                | 6.2      | Fuel oil.                          |
| 3.       | Head        | 100.00       | 54.49           | -----  | 100.00               | 1.6      | Sulfuric acid.                     |
|          | Concentrate | 58.94        | 65.15           | 4.56   | 70.47                | 3.3      | Sulfonated taloel.                 |
|          | Tailing     | 41.06        | 39.19           | -----  | 29.53                | 5.3      | Kerosene.                          |
| 4.       | Head        | 100.00       | 54.63           | -----  | 100.00               | 2.5      | Sulfuric acid.                     |
|          | Concentrate | 56.91        | 65.18           | 5.36   | 67.90                | 3.5      | Oil-soluble petroleum sulfonate.   |
|          | Tailing     | 43.09        | 40.70           | -----  | 32.10                |          |                                    |

the pulp before subjecting it to the magnetic separation.

The invention will be more fully described in conjunction with the following examples in which the purpose is illustrative only and not by way of limitation. All parts are by weight unless otherwise noted.

## EXAMPLE 1

In order to show the effect of magnetic separation alone without the conditioning operation, a sample of a beneficiation plant product containing magnetite, martite, and a quartz gangue was divided into a number of samples. One sample

65

In order to demonstrate that the process may be operated successfully in neutral or alkaline circuit and that conditioning may be conducted at low solids, the following example was carried out:

## EXAMPLE 3

70

Several additional samples of the same ore used in previous examples were treated according to the procedure of Example 2 except that the pulp was directly made up at about 25% solids and the conditioning step carried out at that pulp density. No acidifying agent was used except in the last test. It will be seen that the results 75 compare very favorably with those obtained in

Example 2. The metallurgical results and the reagents are shown in Table III.

Table III

| Product          | Per Cent Wt. | Assay, Per Cent |        | Distrib. Per Cent Fe | Reagents |                             |
|------------------|--------------|-----------------|--------|----------------------|----------|-----------------------------|
|                  |              | Fe              | Insol. |                      | Lbs./ton | Type                        |
| Head.....        | 100.00       | 55.78           | .....  | 100.00               | 2.0      | Sulfonated oleic acid.      |
| Concentrate..... | 66.57        | 66.65           | 3.82   | 79.55                | 7.0      | 22° B6. fuel oil.           |
| Tailing.....     | 33.43        | 34.12           | .....  | 20.45                | .....    | .....                       |
| Head.....        | 100.00       | 55.92           | .....  | 100.00               | 4.0      | Sulfonated refined talcoel. |
| Concentrate..... | 75.12        | 65.28           | 6.44   | 87.69                | 5.3      | Kerosene.                   |
| Tailing.....     | 24.88        | 27.66           | .....  | 12.31                | .....    | .....                       |
| Head.....        | 100.00       | 55.25           | .....  | 100.00               | 5.0      | Sulfuric acid.              |
| Concentrate..... | 60.14        | 65.18           | 5.34   | 70.95                | 4.0      | Oil-sol. pet. sulfonate.    |
| Tailing.....     | 39.86        | 40.27           | .....  | 29.05                | 4.4      | Fuel oil.                   |

EXAMPLE 4

A composite of an iron ore washer plant tailing and a magnetite ore was ground and partially deslimed by hydraulic classification. Two samples of the sands were taken and the first subjected directly to magnetic separation as a pulp of about 20% solids. The second was conditioned for 2 minutes at about 70% solids with 1.8 lbs./ton of sulfuric acid, 3.2 lbs./ton of an oil-soluble petroleum sulfonate, and 5.1 lbs./ton of fuel oil and then was diluted to about 25% solids and subjected to magnetic separation. The magnetic concentrate was diluted to about 20% solids and cleaned magnetically. The results obtained are shown in Table IV.

Table IV

| Test No. | Product        | Per cent Weight | Assay, per cent |        | Distrib. Per cent Fe | 35 |
|----------|----------------|-----------------|-----------------|--------|----------------------|----|
|          |                |                 | Fe              | Insol. |                      |    |
| 1.....   | Head.....      | 100.00          | 24.43           | .....  | 100.00               | 40 |
|          | Slime.....     | 12.29           | 24.85           | .....  | 12.50                |    |
|          | Mag. Conc..... | 20.55           | 67.79           | 4.62   | 57.02                |    |
|          | Cl. Tail.....  | 2.44            | 12.92           | .....  | 1.29                 |    |
|          | Tailing.....   | 64.72           | 11.02           | .....  | 28.19                |    |
|          | (Head.....)    | 100.00          | 24.32           | .....  | 100.00               |    |
| 2.....   | Slime.....     | 11.81           | 25.00           | .....  | 12.14                | 45 |
|          | Mag. Conc..... | 28.46           | 62.23           | 8.36   | 72.82                |    |
|          | Cl. Tail.....  | 3.02            | 9.04            | .....  | 1.12                 |    |
|          | Tailing.....   | 56.71           | 5.97            | .....  | 13.92                |    |

EXAMPLE 5

In order to illustrate the treatment of ores which do not naturally contain a magnetic constituent, the following treatment of a hematite ore was carried out. In the first test, a sample of minus 10 plus 65 mesh ore was admixed with about 16% (by weight) of magnetite and the mixture was conditioned for 2 minutes at high solids with 7.7 lbs./ton of sulfuric acid, 6 lbs./ton of an oil-soluble petroleum sulfonate, and 7.5 lbs./ton of fuel oil. The conditioned pulp was diluted to 25% solids and subjected to magnetic separation. In the second test, only 8% of magnetite was added and only 5.9 lbs./ton of sulfuric acid was used, the procedure being otherwise the same. Illustrative results are shown in Table V.

Table V

| Test No. | Product          | Per cent Weight | Assay, per cent |        | Distrib. Per cent Fe | 70 |
|----------|------------------|-----------------|-----------------|--------|----------------------|----|
|          |                  |                 | Fe              | Insol. |                      |    |
| 1.....   | Head.....        | 100.00          | 53.97           | 13.60  | 100.00               | 75 |
|          | Concentrate..... | 86.15           | 57.66           | 13.60  | 92.04                |    |
|          | Tailing.....     | 13.85           | 31.02           | .....  | 7.96                 |    |
|          | Head.....        | 100.00          | 53.20           | 10.70  | 100.00               |    |
| 2.....   | Concentrate..... | 72.65           | 58.91           | 10.70  | 80.45                |    |
|          | Tailing.....     | 27.35           | 38.02           | .....  | 19.55                |    |

20

A washer tailing from the Mesabi range containing principally hematite and quartz and assaying about 23% Fe was partially deslimed by hydraulic classification and then was mixed with a magnetite concentrate in the ratio of about 3.1 to 1.0. This pulp was then conditioned for 2 minutes at high solids with 7.2 lbs./ton of sulfuric acid, 4.3 lbs./ton of an oil-soluble petroleum sulfonate, and 4.8 lbs./ton of fuel oil; diluted to about 25% solids and subjected to magnetic separation. The concentrate was cleaned once. The results are shown in Table VI.

EXAMPLE 6

30

| Product        | Per Cent Wt. | Assay, Per Cent |        | Distrib. Per Cent Fe |
|----------------|--------------|-----------------|--------|----------------------|
|                |              | Fe              | Insol. |                      |
| Head.....      | 100.00       | 31.54           | .....  | 100.00               |
| Mag. Conc..... | 45.50        | 58.29           | 14.88  | 84.08                |
| Cl. Tail.....  | 2.90         | 8.38            | .....  | 0.77                 |
| Tailing.....   | 51.60        | 9.26            | .....  | 15.15                |

EXAMPLE 7

A New Jersey magnetite-martite ore assaying about 13% iron, the major portion of the iron being present as a non-magnetic oxide, was ground for 12 minutes in a rod mill and then diluted to about 25% solids. This pulp was divided into two samples. The first was directly subjected to magnetic separation and the magnetic concentrate cleaned once magnetically. In the second test, the colloidal fraction was removed by hydraulic classification and the sands conditioned at high solids with 2.0 lbs./ton of sulfuric acid, 2.0 lbs./ton of an oil-soluble petroleum sulfonate, and 1.7 lbs./ton of fuel oil. The conditioned pulp was subjected to froth flotation and the resultant rougher concentrate given a single cleaning by flotation. The cleaned concentrate was then diluted to about 25% solids and subjected to magnetic separation. This produced a high grade concentrate and a relatively high grade middling which itself can be subjected to any further desirable treatment such as tabling and the like. This procedure was used to illustrate the adaptability of the present process in conjunction with standard procedures of froth flotation. The results are shown in Table VII.

Table VII

| Test No. | Product         | Per cent Weight | Assay, per cent |        | Distrib. Per cent Fe |
|----------|-----------------|-----------------|-----------------|--------|----------------------|
|          |                 |                 | Fe              | Insol. |                      |
| 1-----   | Head.....       | 100.00          | 13.70           | -----  | 100.00               |
|          | Mag. Conc.....  | 9.80            | 63.45           | 9.44   | 44.46                |
|          | Cl. Tail.....   | 2.85            | 20.57           | -----  | 4.28                 |
|          | Tailing.....    | 87.55           | 8.02            | -----  | 51.28                |
|          | Head.....       | 100.00          | 13.32           | -----  | 100.00               |
|          | Slime.....      | 6.24            | 6.62            | -----  | 3.10                 |
| 2-----   | Flot. Conc..... | 21.31           | 55.98           | 13.28  | 89.59                |
|          | Cl. Tail.....   | 7.83            | 3.60            | -----  | 2.12                 |
|          | Tailing.....    | 64.62           | 1.07            | -----  | 5.19                 |
|          | Flot. Conc..... | 21.31           | 55.98           | 13.28  | 89.59                |
|          | Mag. Conc.....  | 17.43           | 58.62           | 9.92   | 76.73                |
|          | Mag. Tail.....  | 3.88            | 44.16           | 28.04  | 12.86                |

**EXAMPLE 8**

Another portion of the same ore used in Example 7 was ground and partially deslimed by hydraulic classification to remove the colloidal fraction. By the same treatment used in the second test of Example 7, the sands were then conditioned with various reagents and subjected directly to magnetic separation. The reagents used and the results obtained are shown in Table VIII. It will be seen that the results obtained are superior to those of the direct separation without the conditioning obtained in Test 1 of Example 7.

Table IX

| Test<br>No. | Product        | Per cent<br>Weight | Assay, per cent |        | Distrib.<br>Per cent<br>Fe |
|-------------|----------------|--------------------|-----------------|--------|----------------------------|
|             |                |                    | Fe              | Insol. |                            |
| 1           | Head           | 100.00             | 22.87           | —      | 100.00                     |
|             | Mag. Conc.     | 15.23              | 66.49           | 7.02   | 44.27                      |
|             | Cl. Tail       | 4.59               | 27.68           | —      | 5.56                       |
|             | Tailing        | 80.18              | 14.31           | —      | 80.17                      |
|             | Head           | 100.00             | 23.82           | —      | 100.00                     |
|             | Slime          | 7.36               | 8.60            | —      | 2.66                       |
| 10          | Mag. Conc.     | 31.13              | 64.32           | 9.72   | 84.07                      |
|             | Cl. Tail       | 6.21               | 10.03           | —      | 2.61                       |
|             | Tailing        | 55.30              | 4.59            | —      | 10.56                      |
|             | Head           | 100.00             | 23.58           | —      | 100.00                     |
|             | Slime          | 10.05              | 9.90            | —      | 4.22                       |
|             | Mag. Conc.     | 22.84              | 69.86           | 5.04   | 67.68                      |
| 15 3        | Martite Conc.  | 8.73               | 47.24           | 26.22  | 17.49                      |
|             | Cl. Tail       | 3.80               | 6.60            | —      | 1.04                       |
|             | Tailing        | 54.58              | 4.12            | —      | 9.55                       |
|             | Combined Conc. | 31.57              | 63.60           | 10.90  | 85.17                      |
|             |                |                    |                 |        |                            |
|             |                |                    |                 |        |                            |

I claim:

20 1. A method of concentrating oxidized iron mineral values from mixtures thereof containing acidic gangue and both magnetic and non-magnetic iron oxides, which comprises the steps of making an aqueous pulp of the solids of sufficiently small size to insure liberation of the mineral values, conditioning the aqueous pulp with an agglomerating agent combination comprising a material selected from the group consisting of sulfonated long-chain aliphatic fatty acids, sul-

25

Table VIII

| Test No. | Product   | Per Cent Wt. | Assay, Per Cent |        | Distrib. Per Cent Fe | Reagents |                          |
|----------|-----------|--------------|-----------------|--------|----------------------|----------|--------------------------|
|          |           |              | Fe              | Insol. |                      | Lbs./ton | Type                     |
| 1.       | Head      | 100.00       | 13.38           | -----  | 100.00               |          |                          |
|          | lime      | 6.01         | 6.86            | -----  | 3.08                 | 2.0      | Sulfuric acid.           |
|          | Mag. Conc | 15.61        | 55.83           | 14.98  | 65.11                | 2.0      | Oil-sol. pet. sulfonate. |
|          | Cl. Tail  | 3.80         | 15.11           | -----  | 4.29                 | 1.7      | Fuel oil.                |
|          | Tailing   | 74.58        | 4.94            | -----  | 27.52                |          |                          |
| 2.       | Head      | 100.00       | 13.23           | -----  | 100.00               |          |                          |
|          | Slime     | 6.04         | 7.32            | -----  | 3.34                 | 3.0      | Sulfuric acid.           |
|          | Mag. Conc | 14.64        | 59.84           | 9.90   | 66.23                | 3.0      | Oil-sol. pet. sulfonate. |
|          | Cl. Tail  | 2.84         | 16.50           | -----  | 3.54                 |          |                          |
|          | Tailing   | 76.48        | 4.65            | -----  | 26.89                |          |                          |

**EXAMPLE 9**

A low grade iron ore assaying about 22-23% Fe was crushed and ground, divided into a number of portions and the portions given the following treatments. Portion 1 was diluted with water to about 25% solids, subjected directly to magnetic separation and the concentrate given a single magnetic cleaning. Portion 2 was partially deslimed to remove the colloidal fraction, diluted to 25% solids and conditioned for 1½ minutes with 4.0 lbs./ton of sulfonated refined talloel and 6.2 lbs./ton of No. 2 fuel oil. The pulp was subjected to a magnetic separation and the concentrate therefrom was conditioned without additional reagents for ½ minute and given a magnetic cleaning. The third portion was given the same treatment as the second except that the reagents used were sulfuric acid, 3.0 lbs./ton, and an oil-soluble petroleum sulfonate, 3.0 lbs./ton, and 22° Bé. fuel oil, 4.4 lbs./ton. The rougher concentrate was given a magnetic cleaning. The cleaned concentrate was conditioned for 5 minutes at low solids with 3.0 lbs./ton of soda ash and 0.35 lb./ton of quebracho to release the flocules, and the treated concentrate was then magnetically separated to recover the magnetite. The non-magnetic remainder was designated as the martite concentrate. The results are shown in Table IX.

fonated saponifiable oils of animal and vegetable origin, sulfonated talloel, sulfonated naphthenic acids, petroleum sulfonates of the oil-soluble mahogany acid and water-soluble green acid types obtained in the refining of natural and synthetic

50 obtained in the refining of petroleum lubricating oils, mixtures of these petroleum sulfonates and salts of these materials, together with an unsaponifiable oil, in amount sufficient to insure thorough dissemination of the sulfonated reagent,  
55 and, at least in the case of the petroleum sulfonates, a material selected from the group consisting of acids and materials liberating an acidic substituent in solution, having a dissociation constant greater than  $10^{-7}$  and used in sufficient  
60 amount to produce a pH of about 5.5-1.5; subjecting the conditioned pulp to a magnetic separation whereby a magnetic concentrate is removed comprising the magnetic substituents and a major portion of the desired non-magnetic substituents.

2. A process according to claim 1 in which the magnetic concentrate agglomerate is broken up, and the so treated concentrate is subjected to a magnetic separation whereby a magnetic concentrate comprising the magnetic substituents is removed and at least a part of the magnetic concentrate so removed is admixed with fresh feed prior to the agglomerating operation.

3. A process according to claim 1 in which the aqueous pulp of the mixture to be treated is con-

ditioned with the agglomerating reagent combination under conditions adapted to introduce a finite quantity of minute air bubbles into the pulp but the amount of air introduced is insufficient to produce any appreciable froth concentrate at the surface of the pulp.

4. A process according to claim 1 in which the agglomerating reagent combination comprises fuel oil and a sulfonated fatty acid.

5. A process according to claim 1 in which the agglomerating reagent combination comprises sulfonated talloel and a fuel oil.

6. A process according to claim 1 in which the agglomerating reagent combination comprises a strong inorganic acid, a fuel oil, and a petroleum sulfonate selected from the group consisting of the oil-soluble, mahogany acid and water-soluble green acid types, obtained in the refining of petroleum lubricating oils, mixtures thereof and salts of these sulfonates.

7. A method of beneficiating ores containing oxidized iron mineral values and acidic gangue, the iron mineral values being present as both magnetic and non-magnetic oxides which comprises the steps of making an aqueous pulp of the solids of sufficiently small size to insure liberation of the mineral values, conditioning the aqueous pulp with an agglomerating agent combination comprising a material selected from the group consisting of sulfonated long-chain aliphatic fatty acids, sulfonated saponifiable oils of animal and vegetable origin, sulfonated talloel, sulfonated naphthenic acids, petroleum sulfonates

of the oil-soluble mahogany acid and water-soluble green acid types obtained in the refining of petroleum lubricating oils, mixtures of these petroleum sulfonates and salts of these materials, together with an unsaponifiable oil, in amount sufficient to insure thorough dissemination of the sulfonated reagent, and at least in the case of the petroleum sulfonates a material selected from the group consisting of acids and materials liberating an acidic substituent in solution, having a dissociation constant greater than  $10^{-7}$  and used in sufficient amount to produce a pH of about 5.5-1.5; subjecting the conditioned pulp to a magnetic separation whereby a magnetic concentrate is removed comprising the magnetic substituents and a major portion of the desired non-magnetic substituents.

EARL CONRAD HERKENHOFF.

#### REFERENCES CITED

The following references are of record in the file of this patent:

#### UNITED STATES PATENTS

| Number    | Name     | Date          |
|-----------|----------|---------------|
| 933,717   | Lockwood | Sept. 7, 1909 |
| 1,043,850 | Lockwood | Nov. 12, 1912 |
| 2,069,182 | Hagood   | Jan. 26, 1937 |

#### OTHER REFERENCES

Ref Le Genie Civil Tome XCIII No. 14, pages 328 to 330, Oct. 6, 1928.